

# United States Patent Office

2,861,044

Patented Nov. 18, 1958

1

2,861,044

## POLYPHOSPHATE COMPOSITION CONTAINING TARNISH INHIBITOR

Edgar E. Ruff and Robert E. Dukeshire, Cambridge, Mass., assignors to Lever Brothers Company, New York, N. Y., a corporation of Maine

No Drawing. Application July 8, 1950  
Serial No. 172,776

16 Claims. (Cl. 252—137)

This invention relates to polyphosphate compositions containing tarnish inhibitors, and, more particularly, to detergent compositions containing polyphosphate builders and tarnish inhibitors.

A wide variety of compositions containing polyphosphates have now become well-known and are in general use. It has been found, however, that aqueous solutions of such compositions tarnish copper, and nickel and copper alloys such as German silver (a nickel-zinc-copper alloy) to a variety of shades from yellow to bluish black if permitted to remain in contact therewith for several minutes, especially if the solutions are at elevated temperatures. This is a serious problem in the detergent art, for German silver is frequently used for household articles commonly washed in polyphosphate-containing detergent compositions.

Since detergent compositions containing phosphates, such as sodium orthophosphate, do not cause tarnishing, the difficulty could be avoided by using phosphate builders other than the polyphosphates. This is undesirable, however, because polyphosphates display a synergistic effect with many detergents, and for this reason are highly regarded by the art.

Accordingly, it is an object of the present invention to provide a tarnish inhibitor for polyphosphate compositions.

It is a further object to incorporate with compositions containing polyphosphates a material which will inhibit the tarnishing of metals, and particularly the tarnishing of German silver, by such compositions.

It is a further object of the present invention to provide a detergent composition containing polyphosphate builders and a tarnish inhibitor therefor, which composition will not tarnish metals such as German silver.

The tarnish inhibitors in accordance with the invention are five-membered heterocyclic ring compounds containing in the ring a nitrogen atom and an atom of an element of group VI of the periodic table selected from the group consisting of oxygen and sulfur, spaced from the nitrogen atom in the ring by one carbon atom. The said ring carbon atom bears as a substituent a mercapto radical. Those skilled in the art will recognize these as thiazole, thiazoline, oxazole and oxazoline compounds having a mercapto group substituted at the 2-carbon position. These heterocyclic compounds may be represented by the general structural formula



where X is selected from the group consisting of oxygen and sulfur and Z is a radical or radicals taken in sufficient number to satisfy the free valences of the Nos. 4- and 5-carbon atoms. These carbons have two free valences in oxazoles and thiazoles, and four free valences in oxazolines and thiazolines.

The anti-tarnish activity of these compounds is believed to be due to the presence of an anti-tarnish group,  $\text{—N}=\text{C—X—}$ , group, which may be represented by the following structural formulas:

2

or its tautomeric form, the

$-\text{NH—C—X—}$  group

Z therefore is a substituent which does not react with or inhibit the anti-tarnishing activity of this group, and preferably is selected from the group consisting of hydrogen, oxo oxygen, alkyl, such as methyl, aryl, such as phenyl or diphenyl, and saturated and unsaturated mono and polynuclear alicyclic and heterocyclic rings, such as cyclohexyl or benzene rings condensed with, i. e., sharing two carbon atoms with, the above heterocyclic ring in a polycyclic system. Rings condensed therewith may bear noninterfering substituents, such as halogen, amino, alkyl and aryl groups.

The dotted line bonds in the above formula denote two single bonds, one each at the 4- and 5-carbon atoms, respectively, in oxazolines and thiazolines and one double bond between the 4- and 5-carbon atoms in the oxazoles and thiazoles.

The following compounds are examples of those which have structures within the limits of the above general formula, and are suggested for use as tarnish inhibitors:

(1) 2-mercaptop-4-phenylthiazoline



(2) 2-mercaptopbenzothiazole



(3) 6-amino-2-mercaptopbenzothiazole



(4) 2-mercaptopthiazole



(5) 2-mercaptop-4,5-dimethylthiazole



(6) 2-mercaptopbenzoxazole



(7) 2-mercaptopoxazoline



(8) 2-mercaptopthiazoline



(9) 2-mercaptopthiazoline-4-one



(10) 2-mercaptopoxazole



## (11) 4,4-dimethyl-2-mercaptopoxazoline



## (12) 2-mercaptopcyclohexylthiazoline



Between 0.03% and about 1% of one or a mixture of two or more of these compounds by weight of the polyphosphate inhibits the tarnishing of metals by polyphosphates, even in the presence of synthetic detergents and builders of the type customarily employed in formulating detergent compositions.

The following examples are given for purposes of

to 1% by weight of the polyphosphate) of one of the tarnish inhibitors listed in the following table to a standard commercial detergent, composed of the following ingredients in the proportions specified:

|                                                                                                                                                                                                                                                                                      | Percent |
|--------------------------------------------------------------------------------------------------------------------------------------------------------------------------------------------------------------------------------------------------------------------------------------|---------|
| 5 Magnesium phenylpolypropylene sulfonate                                                                                                                                                                                                                                            | 34      |
| Tetrasodium pyrophosphate and pentasodium tripolyphosphate                                                                                                                                                                                                                           | 48      |
| Other builders, water and inert material                                                                                                                                                                                                                                             | 18      |
| 10 Aqueous solutions containing 5 g. composition in one quart water of 60 p. p. m. hardness were prepared and brought to 165° F. German silver utensils were immersed in these solutions for thirty minutes at 165° F. and then taken out, rinsed lightly with warm water and dried. |         |
| 15 The effectiveness of the tarnish inhibitor in preventing tarnish was noted and rated on the same scale as in Example I. The results were as follows:                                                                                                                              |         |

| Example | Tarnish Inhibitors                                              | Percent Amount of Inhibitor |      |      |       |       |       |
|---------|-----------------------------------------------------------------|-----------------------------|------|------|-------|-------|-------|
|         |                                                                 | 1.0                         | 0.50 | 0.25 | 0.125 | 0.063 | 0.031 |
| 1.      | Phenylbiguanide salt of 2-mercaptopbenzothiazole.               | (1)                         | (1)  | (2)  | —     | —     | —     |
| 2.      | 0-tolyl biguanide salt of 2-mercaptopbenzothiazole.             | —                           | (3)  | —    | —     | —     | —     |
| 3.      | 0-biphenyl biguanide salt of 2-mercaptopbenzothiazole.          | —                           | (1)  | (2)  | —     | —     | —     |
| 4.      | Zinc salt of 2-mercaptopbenzothiazole.                          | —                           | (3)  | (3)  | —     | —     | —     |
| 5.      | Benzyl hexamethylenetetramine salt of 2-mercaptopbenzothiazole. | —                           | (2)  | (3)  | —     | —     | —     |
| 6.      | 6-amino-2-mercaptopbenzothiazole.                               | —                           | (3)  | (3)  | —     | —     | —     |
| 7.      | 2-mercaptop-4,5-dimethylthiazole.                               | —                           | (3)  | (3)  | —     | —     | —     |
| 8.      | 2-mercaptopthiazoline.                                          | —                           | (1)  | (1)  | (1)   | (2)   | (2)   |
| 9.      | 2-mercaptopbenzoxazole.                                         | —                           | (1)  | (1)  | (2)   | (3)   | —     |
| 10.     | 2-mercaptopoxazoline.                                           | —                           | (1)  | (1)  | (1)   | (2)   | (2)   |
| 11.     | 2-mercaptopbenzothiazole.                                       | —                           | (2)  | (2)  | —     | —     | —     |
| 12.     | 2-mercaptopthiazole-4-one.                                      | —                           | (2)  | (2)  | (2)   | (3)   | —     |
| 13.     | 2-hydroxy-4-methylthiazole.                                     | —                           | (5)  | —    | —     | —     | —     |
| 14.     | Benzothiazole.                                                  | —                           | (5)  | —    | —     | —     | —     |
| 15.     | 2-methylbenzothiazole.                                          | —                           | (5)  | —    | —     | —     | —     |
| 16.     | Benzoxazole.                                                    | —                           | (5)  | —    | —     | —     | —     |
| 17.     | 2-methylbenzoxazole.                                            | —                           | (5)  | —    | —     | —     | —     |
| 18.     | 2-methylmercaptopbenzothiazole.                                 | —                           | (5)  | —    | —     | —     | —     |
| 19.     | 4,4-dimethyl-2-mercaptopoxazoline.                              | —                           | (2)  | (2)  | (2)   | (3)   | —     |

illustration of the invention, but the invention is not to be limited thereby.

## Example I

The effectiveness of several typical tarnish inhibitors of the invention with various sodium polyphosphates was determined as follows: 5 g. polyphosphate and 0.25 or 0.063% inhibitor by weight of the polyphosphate were dissolved in 1 quart of water of 60 p. p. m. hardness. The solutions were brought to 165° F. and German silver utensils immersed therein. The solutions were held at that temperature for thirty minutes, after which the utensils were taken from the solution, rinsed lightly with warm water, dried with a cloth, and the amount of tarnish noted. The following were the results:

German silver utensils immersed in a solution of the detergent composition without tarnish inhibitor turned blue-black under the conditions of the above test.

The importance of the mercapto group in the 2-position is demonstrated by the fact that 2-hydroxy-4-methylthiazole (SH replaced by OH), 2-methylmercaptopbenzothiazole (SH replaced by SCH<sub>3</sub>), benzothiazole (SH replaced by H), benzoxazole (SH replaced by H), 2-methylbenzothiazole (SH replaced by CH<sub>3</sub>), and 2-methylbenzoxazole (SH replaced by CH<sub>3</sub>) showed no tarnish protection at a concentration of 0.5%.

## Example II

Detergent solutions were formulated by dissolving 1.7 g. of active component, 2.4 g. of tetrasodium pyrophosphate, and 12.5 mg. of 2-mercaptopthiazoline in one

| Example | Tarnish Inhibitor         | Concentration of Inhibitor, percent | Sodium Polyphosphate |                   |                     |                    |
|---------|---------------------------|-------------------------------------|----------------------|-------------------|---------------------|--------------------|
|         |                           |                                     | Pyrophosphate        | Tri-polyphosphate | Tetra-polyphosphate | Hexa-metaphosphate |
| 1.      | None.                     | —                                   | (5)                  | (5)               | (5)                 | (5)                |
| 2.      | 2-mercaptopbenzothiazole. | { 0.25<br>0.063                     | (2)<br>(2)           | (2)<br>(2)        | —                   | —                  |
| 3.      | 2-mercaptopoxazoline.     | { 0.25<br>0.063                     | (1)<br>(1)           | (2)<br>(2)        | (1)<br>(1)          | (1)<br>(1)         |
| 4.      | 2-mercaptopthiazoline.    | { 0.25<br>0.063                     | (2)<br>(3)           | (1)<br>(3)        | (1)<br>(2)          | (1)<br>(1)         |

Note: (1) indicates barely noticeable tarnish; (2) indicates slight tarnish; (3) indicates moderate tarnish; (4) indicates heavy tarnish; (5) indicates very heavy tarnish.

## Example III

Detergent compositions were formulated by adding 0.015 to 0.50% by weight of the composition (0.03%

quart of water (equivalent in amount of active, builder and inhibitor to 5 g. of the detergent composition of the preceding example plus 0.5% inhibitor by weight

of the polyphosphate) and the same inhibition test was carried out as in the preceding example. Results are given below:

| Active detergent:                                       | Appearance of German silver |
|---------------------------------------------------------|-----------------------------|
| Sodium salt of 1-dodecyloxy-2-propanol-3-sulfonic acid  | (2)                         |
| Sodium lauryl sulfate                                   | (2)                         |
| Sodium salt of lauroyl methyl taurine                   | (2)                         |
| Sodium salt of the sulfoacetamide of aminoethyl laurate | (1)                         |
| Alkyl aryl polyethylene glycol ether                    | (2)                         |
| Polyethylene glycol oleate                              | (1)                         |

As stated, the tarnish inhibitors of the invention are effective in amounts as low as 0.03% of the polyphosphate. The amount required for effective prevention of tarnishing depends in part, of course, upon the extent of protection afforded by the particular inhibitor used, and upon the particular phosphate and its concentration. An amount up to about 1% is satisfactory for most purposes, although larger amounts may be employed, if desired, since a moderate excess of inhibitor is not harmful.

The 2-mercapto substituted inhibitors may be used in the form of their organic amine salts, such as the phenylbiguanide, tolylbiguanide and biphenylguanide salts.

The inhibitors are equally effective in both hard and soft water.

The invention is applicable to compositions containing any alkali metal polyphosphates as a class, such as the tripolyphosphates,  $A_5P_3O_{10}$ , including pentasodium tripolyphosphate and pentapotassium tripolyphosphate, the pyrophosphates  $A_4P_2O_7$ , such as tetrasodium pyrophosphate and tetrapotassium pyrophosphate, the hexametaphosphates ( $AlPO_4$ )<sub>6</sub>, such as sodium hexametaphosphate and potassium hexametaphosphate, and the tetrapolyphosphates  $A_4P_4O_{13}$ , such as hexasodium tetrapolyphosphate and hexapotassium tetrapolyphosphate.

Although the anti-tarnishing agents in accordance with the invention may be incorporated in any compositions containing polyphosphates, they are of particular application to synthetic detergent compositions which contain such phosphates as builders, and which are formulated with either anionic or nonionic detergents. Such detergent compositions should contain conventional proportions of active detergent within the range between 15 and 40%, polyphosphate in an amount between 5 and 50%, based on the total composition and the residue builders and inert materials.

The tarnish inhibitors in accordance with the invention are useful with a wide range of anionic and nonionic synthetic detergents. Of the anionic detergents the phenylpolypropylene sulfonates are particularly noteworthy. These sulfonates are characterized by the following structure:



where R is an alkyl group containing from 9 to 15 carbon atoms and derived from polymerized propylene, and X is an alkali or alkaline earth metal, including ammonium, sodium, potassium, magnesium, barium, calcium and strontium. The ammonium radical, although not a metal in some respects, is generally considered to be a member of the alkali metal family and acts as though it were an alkali metal in these sulfonates. These are known compounds, whose preparation and properties are set forth in U. S. 2,477,383 to Lewis, issued July 26, 1949; they are available in commerce under the trade name "Oronite."

The invention is also applicable to water-soluble alkyl

75

aromatic sulfonic acids, such as those prepared by alkylating benzene or naphthalene with a kerosene fraction followed by sulfonation, aliphatic sulfonic acids, esters of sulfuric acid with aliphatic alcohols of 10 to 18 carbon atoms, particularly those derived by the reduction of coconut oil, palm oil and like long-chain fatty acids, sulfonated castor oil, esters and ethers of isethionic acid, the amides of taurine and N-alkyl taurines, where the alkyl group is a small-chain radical containing up to about 10 carbon atoms, long-chain fatty acid esters and long-chain alkyl ethers of 1,2-dihydroxy propane-3-sulfonic acid and sulfuric acid esters of monoglycerides and glycerol monoethers. The salts of these acids are ordinarily employed.

15 The tarnish inhibitors are also useful with nonionic detergents, such as polyethylene glycol thio and oxy ethers of alkyl phenols, polyethylene glycol esters of long-chain fatty acids and polyethylene glycol ethers of long-chain fatty alcohols.

20 The detergent composition may contain other supplemental builders in addition to the polyphosphate, including alkali metal and alkaline earth metal sulfates, chlorides, silicates, borates, carbonates, metaphosphates, and orthophosphates, such as sodium silicate, magnesium sulfate, sodium carbonate, sodium sulfate, trisodium phosphate, potassium carbonate, sodium orthophosphate, sodium metaphosphate, calcium sulfate, calcium chloride, sodium chloride, sodium borate, potassium metaphosphate and magnesium chloride. The builder should but 25 need not be water-soluble.

In addition to or instead of the above-mentioned supplemental inorganic salts, organic materials such as starch, polyethylene glycols, polyvinyl alcohols and salts of carboxymethylcellulose may be used as builders. It has 30 been found that between about 0.1 and 1% of an alkali metal carboxymethylcellulose increases detergency and sudsing.

The builder mixture is so chosen among alkaline, 35 neutral and acidic salts that the composition obtained in an aqueous 0.14% solution has a pH of 7 or above. Preferably, its pH lies within the range from 7 to about 10 since solutions which are more alkaline may be irritating to the skin and tend to weaken some fabrics, particularly woolens. In general, the alkali metal carbonates are 45 preferred agents for bringing the pH of the solution to a high alkaline value within the preferred range.

The detergent composition is prepared by conventional methods, as by blending the ingredients thereof in an aqueous solution or slurry and then drying the resulting 50 mixture in a spray or drum dryer at elevated temperatures.

The tarnish inhibitor may be added to the detergent composition at any stage of its manufacture, to the finished detergent composition, or to the detergent solution.

55 Compositions containing tarnish inhibitors of the invention do not tarnish copper, or nickel copper alloys such as German silver alloy, Monel metal, coinage nickel, or brass, which normally tarnish when exposed to aqueous solutions containing polyphosphates. It is

60 not possible at this time to explain why the compounds of the invention are effective tarnish inhibitors. However, it has been observed that when a German silver utensil is immersed for a period in a solution of the inhibitor and then immersed in a polyphosphate solution 65 not containing inhibitor only slight tarnishing results. This is taken as an indication that inhibitor is preferentially adsorbed by the metal, and that this is important in tarnish prevention, but of course, such evidence is not conclusive.

Obviously, many modifications and variations may be made in the invention herein set forth without departing from the spirit and scope thereof, and only such limitations should be imposed as are indicated in the appended claims.

The expression "consisting essentially of" as used

herein is intended to refer to the components which are essential to the composition, namely, the tarnish inhibitor and the alkali metal polyphosphate, and the expression does not exclude other components from the composition which do not render it unsuitable for the desired purposes, such materials being, for instance, detergents, other builders, such as sodium silicate and sodium carbonate, carboxymethylcellulose, minor quantities of impurities, etc.

All parts and percentages in the specification and 10 claims are by weight. Proportions of inhibitor are based on the weight of the polyphosphate unless otherwise indicated.

We claim:

1. A composition comprising a water-soluble polyphosphate which in aqueous solution tarnishes copper and copper and nickel alloys and a tarnish inhibitor in an amount to lessen the tarnishing action of the polyphosphate and having the general formula



where X is selected from the group consisting of oxygen and sulfur and Z is a radical taken in sufficient number to satisfy the free valences of the 4- and 5-ring carbon atoms and is selected from the group consisting of hydrogen, oxo oxygen, alkyl, aryl and saturated and unsaturated mono and polynuclear alicyclic and heterocyclic rings condensed therewith.

2. A composition in accordance with claim 1 in which the tarnish inhibitor is a thiazole.

3. A composition in accordance with claim 1 in which the tarnish inhibitor is a thiazoline.

4. A composition in accordance with claim 1 in which the tarnish inhibitor is an oxazole.

5. A composition in accordance with claim 1 in which the tarnish inhibitor is an oxazoline.

6. A composition in accordance with claim 2 in which the tarnish inhibitor is 2-mercaptop-4,5-dimethyl thiazole.

7. A composition in accordance with claim 3 in which the tarnish inhibitor is 2-mercaptopthiazoline.

8. A composition in accordance with claim 4 in which the tarnish inhibitor is 2-mercaptopbenzoxazole.

9. A composition in accordance with claim 5 in which the tarnish inhibitor is 2-mercaptopoxazoline.

10. A nonsoap detergent composition consisting essentially of an active organic detergent, a water-soluble polyphosphate which in aqueous solution tarnishes copper and copper and nickel alloys, and a tarnish inhibitor in an amount to lessen the tarnishing action of the polyphosphate and having the general formula



where X is selected from the group consisting of oxygen and sulfur and Z is a radical taken in sufficient number to satisfy the free valences of the 4- and 5-ring carbon atoms and is selected from the group consisting of hydrogen, oxo oxygen, alkyl, aryl and saturated and unsaturated mono and polynuclear alicyclic and heterocyclic rings condensed therewith.

11. A detergent composition in accordance with claim 10 in which the tarnish inhibitor is 2-mercaptopthiazoline.

12. A detergent composition in accordance with claim 10 in which the tarnish inhibitor is 2-mercaptopbenzoxazole.

13. A detergent composition in accordance with claim 10 in which the detergent is sodium phenyl polypropylene sulfonate.

14. A nonsoap detergent composition consisting essentially of an alkali metal alkyl aryl sulfonate detergent, a water-soluble polyphosphate which in aqueous solution tarnishes copper and copper and nickel alloys and a tarnish inhibitor in an amount to lessen the tarnishing action of the polyphosphate and having the general formula



where X is selected from the group consisting of oxygen and sulfur and Z is a radical taken in sufficient number to satisfy the free valences of the 4- and 5-ring carbon atoms and is selected from the group consisting of hydrogen, oxo oxygen, alkyl, aryl and saturated and unsaturated mono and polynuclear alicyclic and heterocyclic rings condensed therewith.

15. A detergent composition consisting essentially of an alkali metal phenyl polypropylene sulfonate detergent, tetrasodium pyrophosphate and a tarnish inhibitor in an amount to lessen the tarnishing action of the polyphosphate and having the general formula



where X is selected from the group consisting of oxygen and sulfur and Z is a radical taken in sufficient number to satisfy the free valences of the 4- and 5-ring carbon atoms and is selected from the group consisting of hydrogen, oxo oxygen, alkyl, aryl and saturated and unsaturated mono and polynuclear alicyclic and heterocyclic rings condensed therewith.

16. A detergent composition consisting essentially of an alkali metal phenyl polypropylene sulfonate detergent, pentasodium tripolyphosphate and a tarnish inhibitor in an amount to lessen the tarnishing action of the polyphosphate and having the general formula



where X is selected from the group consisting of oxygen and sulfur and Z is a radical taken in sufficient number to satisfy the free valences of the 4- and 5-ring carbon atoms and is selected from the group consisting of hydrogen, oxo oxygen, alkyl, aryl and saturated and unsaturated mono and polynuclear alicyclic and heterocyclic rings condensed therewith.

#### References Cited in the file of this patent

#### UNITED STATES PATENTS

|    |           |           |               |
|----|-----------|-----------|---------------|
| 65 | 1,773,024 | Chapman   | Aug. 12, 1930 |
|    | 2,160,293 | Shoemaker | May 30, 1939  |
|    | 2,238,651 | Keenen    | Apr. 15, 1941 |
|    | 2,327,323 | Teeters   | Aug. 17, 1943 |
|    | 2,419,805 | Wegst     | Apr. 29, 1947 |
|    | 2,575,576 | Bacon     | Nov. 20, 1951 |
| 70 | 2,618,603 | Schaefier | Nov. 18, 1952 |
|    | 2,618,605 | Schaefier | Nov. 18, 1952 |